# EUROPEAN PATENT SPECIFICATION

(11) **EP 1 478 873 B1**
(45) Date of publication and mention of the grant of the patent: **06.06.2012**
(21) Application number: 03704191.0
(22) Date of filing: 12.02.2003
(51) Int. Cl.: F17C 1/16

(54) **THIN-WALLED LINER FOR HIGH-PRESSURE VESSELS**
DÜNNWANDIGER LINER FÜR HOCHDRUCKBEHÄLTER
CHEMISE A MINCE PAROI DESTINEE A DES CUVES HAUTE PRESSION

(30) Priority: 15.02.2002 CZ 20020585
(43) Date of publication of application: 24.11.2004
(73) Proprietor: KOMPOZIT - PRAHA s.r.o., 330 02 Dysina 298 (CZ)
(72) Inventor: Koldybaev, Sergei Glebovich, 169 00 Praha 6 (CZ); Lukiyanets, Sergei Vladimirovich, 169 00 Praha 6 (CZ); Moroz, Nikolai Grigorievich, 169 00 Praha 6 (CZ); Rezaev, Mikhail Sergeevich, 169 00 Praha 6 (CZ)
(74) Representative: Langrova, Irena
(86) International application number: PCT/CZ2003/000010
(87) International publication number: WO 2003/069217

(56) References cited:
- EP-A- 0 333 013
- WO-A-01/31253
- US-A- 5 287 987
- US-A- 5 287 988
- US-A- 5 494 188
- US-A1- 2002 175 168

## Description

### Field of technology

This invention involves high-pressure vessels whose core is made of a composite material and lined with hermetic liner on the inside.

### Current state of technology

These are vessels intended for storage and transportation of liquid media, i.e. liquids and gases, under pressure, whose core is made of a composite material and lined with a hermetic layer - liner - on the inside; depending on the type and nature of the liquid medium contained in the vessel, the liner is made of thermoplastics, aluminum or stainless steel. This hermetic enclosure - liner - usually has a sleeve of the same material as the material used for the liner. This sleeve enters the axial socket channel, located in the vessel core, with its whole length during production; a socket is located inside the sleeve, equipped with a stop valve of any suitable type.

These vessels are usually exposed to multiple cyclic high-pressure loads. That is why special attention is paid in such vessels to the material of the hermetic enclosure - liner and the hermetic capacity of the sleeve in the axial socket channel to prevent leakage of the liquid medium or failure of the hermetic vessel.

Attempts to make pressure vessels using polyethylene and a device for sealing the enclosure sleeve in the socket channel of the high-pressure vessel are known.

High-pressure vessels with a core of composite material with an installed socket that is located along the whole length of the axial socket channel and in contact with its inner surface is of special use; inside the sleeve, coaxially to the socket channel, a centrally placed socket is placed - a pressure sleeve of the enclosure layer on the inner surface of the socket channel that has at least one circular or screw protrusion on the side of the vessel core's cavity, recliner against the enclosure sleeve with which it interacts for the purposes of sealing the sleeve - see for example file GB 1023011 A, 16.03.66, F 17 C1/16 and EP 0 333 013, and WO01/31253.

It turns out, however, that the mentioned means are still insufficient for sealing high-pressure vessels because the changes in the socket outlet spacing at high pressure are within the range of flexible deformation at the same time when the value of liquidity of the material of the hermetic enclosure - liner and its sleeve is significantly higher; this discordance in deformation is a basic reason for the vessel's lack of leak tightness at high pressure loads.

Attempts to manufacture pressure vessels with a hermetic device and a liner is specified in the published invention application EP 0300931 A1, F 17 C1/16, which describes a high-pressure vessel with a core of composite material, a flange, installed at the production stage, on the socket of the axial channel and a threaded plug at the outlet, located along the whole length of the channel all the way down in the threaded plug of the inner hermetic enclosure's sleeve, and with a centrally placed sleeve incorporating a stop valve, installed coaxially to the socket channel, which presses the enclosure sleeve to the inner surface of the axial socket channel and is connected to the threaded socket plug with threading.

A similar solution is specified in patents WO 99/27293, WO 99/13263 and US 4,925,044.

At high pressures of the liquid medium that fills the cavity of the vessel core, however, reliable leak tightness of the connection between the enclosure - liner and the outlet sleeve is still not achieved, especially in the place of its contact with the inner surface of the socket channel and with the outer surface of the socket, mostly due to the above-mentioned reasons.

Patent RU 2150634 describes a solution that, to a large extent, removes the above-mentioned shortcomings by creating a reliable device for sealing the sleeve of the inner enclosure - liner in the vessel socket, subject to substantially higher periodicity of high-pressure load.

This task is solved by using a device for sealing the sleeve of the inner enclosure - liner in the socket of the high-pressure vessel with a core of composite material that is lined on the inside with a hermetic enclosure with a sleeve containing a socket with an axial channel, installed in the core, an enclosure sleeve, located along the whole length of the channel, and a socket with a stop valve, located inside the sleeve, coaxially to the socket channel. In line with the description, a circular cavity is created between the enclosure sleeve and the socket, with a sealing material placed in it; the sealing material is pressed in the direction of the axis by pressure from the liquid medium in the cavity of the vessel core and interacts in the radial direction outwards on the inner surface of the enclosure sleeve in the socket channel.

In the most appropriate form of implementation of the solution given in patent RU 2150634, the protruding socket at the end in the direction of the cavity in the vessel core has a flange, and the socket at its loose end protruding from the vessel core - protruding inside and adjoining to the surface of the socket has a flange; both flanges serve for closing from the front side of the circular cavity in which the sealing material is placed.

In this way, it is possible to make a conclusion on the proposed solution under patent RU 2150634 that in the design of the device under that patent, the sealing in the circular chamber is permanently verified by axial load under pressure of the liquid medium and thanks to the volume pliability of the material continuously exerts a force in the radial direction outwards on the sleeve of the enclosure - liner, pressing it tightly to the inner surface of the axial socket channel and securing its reliable tightness.

In this case, however, reliable sealing of the enclosure - liner and the socket is not once again secured completely because it is a general shortcoming of this design solution and earlier design solutions of pressure vessels that amorphous thermoplastics, e.g. polyethylene, are used as materials for the enclosure - liner; thermoplastics have high visco-elastic deformability, low gas permeability coefficient virtually for all technical gases; in case of high pressure, their main shortcoming is loss of strength during decompression, i.e. the so-called Keson disease.

### Summary of the invention

The invention's purpose is to create a more reliable solution of the design of the hermetic enclosure - liner and a solution of the sealing of the sleeve in the inner enclosure - liner in the vessel socket, subject to significantly higher periodicity of high-pressure load.

This task was solved using the proposed design of hermetic liner made of an amorphous thermoplastic material, containing a central cylinder part and two faces, with a socket installed in one of them.

In line with the invention, the thickness of face and central-part walls of the liner is in the proportion of 0,001 - 0,01 of the maximum diameter of the liner and the height of the liner faces is in the proportion of 0,3 - 0,4 of the maximum diameter of the liner; The main part of the amorphous material contains crystalline thermoplastics, with the crystallization temperature of 100 to 280°C, measured using differential scanner calorimetry (DSC) at heating speed of 10°C per minute and the shine of its surface measured under DIN 67530 at the measurement angle of 20° shall be more than 90°.

The most reliable form of implementation of the invention is when the crystalline thermoplastics in the face and central walls of the liner have a crystallinity of 5 to 15° of weight.

It is also a reliable form of implementation if the crystalline thermoplastics in the liner sleeve container have a crystallinity of 75 to 99% of weight.

In the most reliable form of implementation, the crystalline thermoplastics are selected from a group that contains polyethyleneterephthalate, polybutadieneterephthalate, cycloolefin polymer and cycloolefin copolymer.

There is one more form of implementation of the invention in which standard viscosity SV (DCE) of the crystalline thermoplastics, measured under DIN 53728 in a 50:50 mixture of phenol and 1,2-dichlorobenzol, is within 75 to 85%; it is between 800 and 1,800 in dichloroacetic acid.

Another suitable form of implementation is when the impact value of the material in its amorphous state, measured by the Izod method in line with ISO 180/1A, is 2 to 8 kJ per m.

In one example of this solution, it is assumed that polyethyleneterephthalate is used as crystalline thermoplastics, with a temperature of sufficient, i.e. cold crystallization between 120 and 160°C.

In one example of this solution, it is assumed that the crystalline thermoplastics of the liner contain at least one ultraviolet stabilizer selected from 2-hydroxibenzotriazole and triacine.

It is desirable that no fissure appears during any change in the impact value of the crystalline thermoplastics under Sharp in line with ISO 179/1D.

### Brief description of the drawings

The invention is described in greater detail in the mentioned examples of arrangement, with reference to drawings. Figure 1 shows an overall view of the high-pressure vessel in a longitudinal section, with hermetic solution of the socket. Figure 2 is a magnified view of one solution variant from figure 1 in accordance with the invention in a longitudinal section.

### Detailed description of the preferred embodiments

An analysis of basic properties of some of the most widely used thermoplastics as given in table 1 shows that based on the requirements on gas permeability and strength for the purposes of use as a liner material, polyethyleneterephthalate is the most suitable material in terms of strength, deformation characteristics and gas permeability in the crystalline thermoplastics class.

| Polymer name | State | Tensile strength limit MPa | Relative elongatio n when impaired % | Water vapor permeability g/m² | Oxygen, permeability cu. cm / (sq.m·atm) in 24 hours | Melting temperature °C |
|---|---|---|---|---|---|---|
| PENP | Amorphous | 9 - 17 | 500 | 15 - 20 | 6,500 - 8,500 | 102 - 105 |
| PEVP | Amorphous | 17 - 35 | 300 | 5 | 1,600 - 2,000 | 125 - 137 |
| PP | Amorphous | 41 | 300 | 10 - 20 | 370 | 160 - 176 |
| PVC, non-plasticized | Amorphous | 45 - 55 | 120 | 30 - 40 | 150 - 350 | 150 - 220 |
| PVIC | Amorphous | 48 - 137 | 20 - 40 | 1.5 - 5.0 | 8 - 25 | 220 |
| OPS | Amorphous | 62 - 73 | 20 | 70 - 150 | 4,500 - 6,000 | 180 |
| PA | Amorphous | 69 - 97 | 250 - 400 | 40 - 80 | 500 | 225 |
| PET | Amorphous | 150 - 180 | 70 - 110 | 25 - 30 | 40 - 50 | 250 - 260 |
| PET | Crystalline | 190 - 260 | 20 - 30 | 2, 5 - 15 | 2 - 20 | 250 - 260 |
| PK | Amorphous | 59 | 75 | 77 - 93 | 4,500 | 220 - 270 |
| AC | Amorphous | 49 - 83 | 15 - 45 | 100 - 320 | 2,000 - 3,000 | |
| Cellulose hydrate | Amorphous | 48 - 110 | 15 - 25 | 5 - 15 | 670 | |

where
PENP - polyethylene with low specific gravity;
PEVP - polyethylene with high specific gravity;
PP - polypropylene;
PVC - polyvinyl chloride;
PVIC - polyvinylidene chloride;
OPS - oriented polystyrene;
PA - polyamide;
PET - polyethyleneterephthalate;
PK - polycarbonate;
AC - cellulose acetate.

When designing pressure vessels, a certain amount of escaping, i.e. diffusing gas for a specified period of its use is usually permissible. For example the requirement under EN 12245 is 0.25 cm per liter per hour.

The thickness of face walls and cylinder-part walls can be determined on the basis of $δ \geq k * P * S * t / ΔV$
where Δ V - escape volume
k - gas permeability coefficient of the material used P - operating pressure of the gas in the pressure vessel
S - surface area on which gas is leaking
t - time of use of the gas pressure vessel
δ - thickness of the liner wall in the pressure vessel

It is obvious from average reference characteristics of various thermoplastics specified in the table that to secure the requirements on gas permeability, specified in various standards, such as EN 12245 and NGV-4, the wall thickness of the face and the central part of the liner of crystalline thermoplastics should be between 0.001 and 0.01 of the maximum liner diameter and is distinctly lower than the thickness of other types of thermoplastics, e.g. 100 times than polyethylene. Because of the small thickness of liner walls and low gas permeability in case of use of crystalline thermoplastics, loss of strength of the thermoplastics during liner decompression is excluded.

Crystallization of thermoplastics on faces and the cylinder part of the liner with the volume of 5 to 15 weight per cent, with the crystallization temperature between 100 and 280°C, measured using differential scanner calorimetry (DSC) with the heating speed of 10 °C per minute, allows to largely reduce gas permeability through the liner wall, subject to keeping their deformation properties.

As shown in fig. 1 in one of the examples of implementation of high-pressure vessels, core 1 of composite material contains an enclosure in the form of a multiple-layer shell whose layers are made by winding interbreeding threads of glass fiber, soaked in polymer binder in one direction. During production, coaxially positioned flange 2 and flange 3 with socket 4 are wound in this core 1 for the purpose of connection of cavity 5 of core 1 with the surrounding space; vessel core 1 is lined with hermetic liner 6 on the inside, made of crystalline thermoplastics.

As shown in fig. 2 in one of the variants of arrangement of the feeding socket, liner 6 that covers the inside of core 1 has sleeve 7 positioned along the whole length of axial channel 8 of socket 4, adjoined to its inner surface 9. Centrally positioned socket 10 is placed inside sleeve 7, coaxially to the sleeve and socket 4; socket 10 has a flange protruding on the surface at the end in the direction of cavity 5 of vessel core 1; flange 11 of socket 10 adjoins with its circular surface 12 to inner surface 13 of sleeve 7 of liner 6. The diameter of flange 11 equals inner diameter of sleeve 7 of liner 6.

Socket 4 is, at its free outlet end from core 1, fitted with internally protruding flange 14, adjoining with its circular surface 15 to outer surface 16 of socket 10.

In consequence, there is a circular, concentrically positioned cavity 17, covered from the front by flange 11 of socket 10 and flange 14 of socket 4, between sleeve 7 of liner 6 and socket 10. Sealing 18 is placed inside cavity 17 and fills its whole volume; during axial movement of socket 10 by the pressure on its flange 11 by the liquid medium in cavity 5 of core 1, sealing 18 is compressed axially and acts in the radial direction outwards on internal surface 13 of sleeve 7 if liner 6, pushing it by force against inner surface 9 of axial channel 8 of socket 4, thus sealing sleeve 7 in channel 8 of socket 4.

In case of high pressure in the cavity of core 1 of the vessel, there is pressure in circular cavity 17 that is 3 to 5 times higher than the pressure in cavity 5.

That is why it is necessary to increase the strength of the thermoplastics and its low creep in the zone of contact between sealing 18 and sleeve 7. This is solved by way of crystallization of the liner sleeve. Crystallization of the thermoplastics in the volume of 75 to 99 weight per cent in the zone of the feeding socket allows to increase the strength of the thermoplastics in the given zone and reduce the characteristics of continuous creep of the crystalline thermoplastics several times. This will in turn result in increased operating characteristics of the connection node.

In case of load on the pressure vessel by pressure on the surface, there is a friction stress between the composite and the liner that depends on the level of purity of the liner surface, which can be in turn determined based on the shine in accordance with DIN 67530. Surface shine of over 90 under DIN 67530 is the most acceptable option for the given variant of liner that employs crystalline thermoplastics.

In order to achieve the above-mentioned characteristics of crystalline thermoplastics, it is the most convenient to use thermoplastics with standard viscosity, measured in line with DIN 53728 in a 50:50 mixture of phenol and 1,2-dichlorobenzol, so that it is within 75 to 85%; or in dichloroacetic acid that is between 800 and 1,800.

In order to avoid local damage in zones of stress concentration and deformation, it is the most convenient to use thermoplastics whose impact value in amorphous condition, measured by the Izod method under ISO 180/1A, is over 2 to 8 kJ per m; it is desirable that no fissure appears in case of change in the impact value of the crystalline thermoplastics through the Sharp method under ISO 179/1D.

Due to reasons of general availability, polyethyleneterephthalate is the most widely used well-known thermoplastic material, well adjusted for processing in one of the reasonable options of design of the liner; this material shall have a temperature of sufficient, i.e. cold crystallization between 120 and 160°C which, to improve aging properties in natural conditions, contains at least one ultraviolet stabilizer selected from 2-hydroxibenzotriazole and triacine.

To provide for strength of the pressure vessel made of composite, the face profile on the pressure vessel shall be selected with respect to uniform tension of reinforcing composite fibers along the whole length of the meridian. To secure this solution using thin-walled deformable liner, it is necessary that the maximum height of the liner face profile is between 0,3 and 0,4 of the maximum liner diameter. In this case, i.e. winding of reinforcing fibers and subsequent overfilling of the liner, pressure vessel faces assume the shape of the optimum profile that secures uniform tension of all reinforcing fibers of the used composite.

The functionality of the high-pressure vessel involves its filling with a liquid medium, i.e. liquid or gas, up to the required level of pressure, its storage, transportation, discharge, subsequent re-filling and consumption of the liquid medium, i.e. repeated actions and operations with multiple cyclic loads.

The function of the solution in the invention was described in the description of variants of arrangement and is understandable for experts in the given field, and therefore does not require any further special explanation.

The invention is not limited by the above-mentioned forms of implementation that are only given to illustrate the invention; it can be modified in the patent claims.

### Industrial applications

The proposed solution gives a real possibility to use high-pressure vessels of composite material and with an inner hermetic liner. Production and testing of high-pressure vessels with the proposed liner for sealing confirmed their high reliability and efficiency.

## Claims

1. Thin-walled liner of amorphous material mounted in high-pressure vessels of composite material, e.g. fiberglass, the vessel comprising a central cylinder part and two faces, with a socket (4) in one of them, the liner having a sleeve positioned along the whole length of axial channel of the socket ***characterized by the*** fact that the thickness of face and central-part walls of the liner (6) being in the proportion of 0.001 - 0.01 of the maximum diameter of the liner (6)
and the height of the liner faces being in the proportion of 0,3 - 0,4 of the maximum diameter of the liner (6),
wherein material of the liner (6) - crystalline
thermoplastics being crystalline in the range of 5 to 15 weight per cent and the sleeve wall in liner faces being crystalline in the range of 75 to 99 weight per cent and crystalline thermoplastics have the crystallization temperature of 100 to 280°C, measured using differential scanner calorimetry (DSC), at the heating speed of 10°C per minute and the surface shine of over 90 at the measuring angle of 20°.

2. Liner under claim 1, ***characterized by the*** fact that the standard viscosity SV (DCE) of the crystalline
thermoplastics in a 50:50 mixture of phenol and 1,2-dichiorobenzol being between 75 to 85%; being between 800 and 1,800 in dichloroacetic acid.

3. Liner under claims 1 to 2, ***characterized by the*** fact that the crystalline thermoplastics being selected from a group containing polyethyleneterephthalate, polybutadienterephthalate, cycloolefin polymers and
cycloolefin copolymers.

4. Liner under claims 1 to 3, ***characterized by the*** fact that that no fissure appears during the Sharp impact value test of the crystalline thermoplastics.

5. Liner under claims 1 to 4, ***characterized by the*** fact that the impact value of the material in its amorphous state, measured using the Izod method, being 2 to 8 kJ per meter.

6. Liner under claims 1 to 5, ***characterized by the*** fact that the crystalline thermoplastics being polyethyleneterephthalate with the temperature of sufficient, i.e. cold crystallization being between 120 and 160°C.

7. Liner under claims 1 to 6, ***characterized by the*** fact that the crystalline thermoplastic material of the liner containing at least one ultraviolet stabilizer, selected from 2-hydroxibenzotriazole and triacine.

## Patentansprüche

1. Dünnwandiger Liner aus amorphem Material, untergebracht in Hochdruckbehältern aus Kompositionsmaterial, z.B. aus Fiberglass, wobei der Behälter einen Zentralzylinderteil und zwei Stirnteile beinhaltet, mit einem Stutzen (4) in einem deren, wobei der Liner einen entlang der ganzen Länge des Axialkanals des Stutzens untergebrachten Rohransatz hat, ***dadurch gekennzeichnet,* dass** die Dicke des Stirnteils und der Wand des Zentralteils des Liners (6) im Verhältnis von 0,001- 0,01 des größten Durchmessers des Liners (6) ist,
und die Höhe der Linerstirnteile im Verhältnis von 0,3 - 0,4 des größten Durchmessers des Liners (6) ist,
wobei das Material des Liners (6) - kristallischer Thermoplast -im Bereich von 5 bis 15 Gewichtsprozent kristallisch ist und die Rohransatzwand in Linerstirnteilen im Bereich von 75 bis 99 Massenprozent kristallisch ist und der kristallische Thermoplast die Kristallisationstemperatur von 100 bis 280°C hat, gemessen mit Differenzscannermethode (DSC), bei der Erwärmungsgeschwindigkeit von 10°C per Minute und Oberflächenglanz über 90 unter dem Messwinkel von 20°.

2. Der Liner dem Anspruchs 1 zufolge, ***dadurch gekennzeichnet,* dass** die Standardviskosität SV (DCE) des kristallischen Thermoplasts in der Mischung von 50:50 des Phenols und 1,2-Dichlorbenzols zwischen 75 und 85 % ist; sie ist zwischen 800 und 1800 in der Dichloraceticsäure.

3. Der Liner den Ansprüchen 1 und 2 gemäß, ***dadurch gekennzeichnet,* dass** der kristallische Thermoplast aus der die Polyethylenterephtalate, Polybutadienterephtalate, Zycloolephinpolymere und Zycloolephicopolymere beinhaltenden Gruppe gewählt wird.

4. Der Liner den Ansprüchen 1 bis 3 gemäß, ***dadurch gekennzeichnet,* dass** während der Schlagzähigkeitprüfung des kristallisches Thermoplasts nach Sharp keine Risse entstehen.

5. Der Liner nach den Ansprüchen 1 bis 4, ***dadurch gekennzeichnet,* dass** die Schlagzähigkeit des Materials im amorphen Zustand, gemessen mit der Izod-Methode, 2 bis 8 kJ per Meter ist.

6. Der Liner den Ansprüchen 1 bis 5 gemäß, ***dadurch gekennzeichnet,* dass** der kristallische Thermoplast das Polyethylenterephtalat mit hinreichender Temperatur, d.h. kalter Kristallisation, zwischen 120° bis 160°C ist.

7. Der Liner nach den Ansprüchen 1 und 6, ***dadurch gekennzeichnet,* dass** der kristallische Thermoplastmaterial des Liners mindestens einen aus 2-Hydroxibenzotrialzole und Triacine gewählten Ultraviolettstabilisator beinhaltet.

## Revendications

1. Chemise à paroi mince de matériau amorphe installée dans des cuves haute pression de matériau composé, par exemple le fibreglass, le cuve contenant la partie cylindrique centrale et deux faces, avec le goulot (4) dans l'un d'eux, la chemise ayant un manchon posé le long de toute la longueur du canal du goulot, ***caractérisée par le fait* que** l'épaisseur de la face et des parois de la partie centrale de la chemise (6) sont en proportion de 0,001 - 0,01 du diamètre maximum de la chemise (6)
et la hauteur des faces de la chemise est en la proportion de 0,3 - 0,4 du diamètre maximum de la chemise (6),
pourtant que le matériau de la chemise (6) - le thermoplastique cristalline - est cristalline dans l'étendue de 5 jusqu'à 15 pour-cent de masse et les parois du manchon dans les faces de la chemise sont cristalline en l'étendue de 75 jusqu'à 99 pour-cent de poids, et le thermoplastique cristalline ont la température de cristallisation de 100 jusqu'à 280°C, mesurée à l'aide de la calorimétrie différentielle de scanner (DSC), à la vélocité du chauffage de 10°C en une minute et l'éclat de surface au-dessus de 90 à l'angle de mesurage de 20°.

2. La chemise selon le revendication 1, ***caractérisée par le fait* que** la viscosité standard SV (DCE) du thermoplastique cristalline dans le mélange 50:50 du phénol et du 1,2-dichlorobenzol est entre 75 jusqu'à 85 %; elle est entre 800 et 1,800 dans l'acide dichloroacetique:

3. La chemise selon les revendications 1 et 2, ***caractérisée par le fait* que** le thermoplastique cristalline est choisi du groupe contenant polyéthylèneterephtalate, polybutadienterephtalate, polymères cyclooléphines et copolymères cyclooléphines.

4. La chemise selon les revendications 1 jusqu'à 3, ***caractérisée par le fait* que** aucune fissure apparaît pendant l'essai de la résilience selon Sharp.

5. La chemise selon les revendications 1 jusqu'à 4, ***caractérisée par le fait* que** la valeur de la résilience du matériau en état amorphe, mesurée par la méthode d'Izod, est 2 jusqu'à 8 kJ pour mètre.

6. La chemise selon les revendications 1 jusqu'à 5, ***caractérisée par le fait* que** le thermoplastique cristalline est polyéthylèneterephtalate avec la température de cristallisation satisfaisante, c'est froide, est parmi 120° et 160°C.

7. La chemise selon les revendications 1 jusqu'à 6, ***caractérisée par le fait* que** le matériau thermoplastique cristalline de la chemise contient tout au moins un stabilisateur ultra-violet choisi de 2-hydroxybenzotriazole et triacine.
